

J. CORSON.  
COLLECTING GOLD, SILVER, AND OTHER METALS FROM THEIR ORES.  
No. 77,591. Patented May 5, 1868.



*Witnesses:*  
J. C. Connolly.  
H. Garrett.



*Inventor:*  
John Corson

# United States Patent Office

JOHN CORSON, OF WASHINGTON CITY, DISTRICT OF COLUMBIA.

*Letters Patent No. 77,591, dated May 5, 1868.*

## IMPROVEMENT IN COLLECTING GOLD, SILVER, AND OTHER METALS FROM THEIR ORES.

The Schedule referred to in these Letters Patent and making part of the same.

### TO ALL WHOM IT MAY CONCERN:

Be it known that I, JOHN CORSON, of Washington city, District of Columbia, have invented a new Process for Collecting Gold, Silver, and Copper from their Ores, and aluminum from clay and spar; and I do hereby declare that the following is a full and exact description thereof, reference being had to the accompanying drawings, and to the letters of reference marked thereon.

To enable others skilled in the art and mystery of mining to make use of my invention, I will proceed to describe the process, and necessary means to be used in the practice of it, and the necessary tools and machinery properly belonging to it.

I use two machines, auxiliary to each other, in order to complete the process of crystallization and amalgamation of the metals found in the ores. In one, I use independent currents of electricity, of sufficient intensity to crystallize the metals sought for in the ores. In the other, the amalgamator, I use no electricity whatever. Both machines must be insulated from earth-currents by glass pillars or globes, or other non-conducting substance.

The crystallizer, Sheet No. 1, is built as follows: A tub or pan, of wood or iron, of suitable size, (say eight or ten feet in diameter and two or three feet high,) is constructed. If the pan is of wood, a false bottom of glass, one and a half or two inches thick, or of well-burned and glazed tiles, is provided.

The pan is set on a suitable non-conducting substance, as glass pillars or balls, as shown at B. A glass-shaft, G, is used to propel the mixing-wheels, or any other means as effectual, to insulate the pan from earth-currents.

Four or eight arms, D, are attached to and are driven by the shaft. The arms carry the mixing-wheels through the pulp. The mixing-wheels E E' are made of wood, twenty-four to thirty inches diameter, and two to three inches thick, fastened to the arms by any suitable device. The face of the wheels is covered with a metal tire, and are arranged in pairs. One half of the wheels (numerically) are covered with one kind of metal tire, and the other half have a different metal tire, so that when arranged in the pan they will be in pairs, as set forth in the drawing, C representing one kind of metal and Z the other kind, as copper and zinc, in this wise: Beginning at the outer end of one arm, and looking toward the shaft, the first wheel is covered with the metal, C, the second wheel is covered with the metal, Z, and so on alternating to the end of the arm next the shaft. On the next arm the first metal is Z, the second is C, &c.

I now connect C on the first arm to Z on the second arm with an iron, copper, or other suitable metallic rod, F. At each end of this metallic rod is a small friction-roller, H H', of same metal as the rod, resting on the tire of the wheels, thus forming a metallic connection between the upper side of each pair of wheels, then place a proper conducting-fluid in the pan, as salt, or very dilute acid, and the battery is ready for operation.

To put this pan in use as a crystallizer: First, the raw ore must be crushed, and by a rubbing process, as an arastre, reduced to an impalpable powder; then a sufficient quantity of this prepared ore is put into the pan; then a proper amount of salt or dilute acid, mixed with soft water, must be put on the ore in the pan, rendering it a semi-fluid pulp. As soon as any one pair of wheels are wet with this fluid compound, electricity is generated, and currents are established between each pair of wheels, causing crystallization immediately to commence.

A slow motion is now given to the wheels, by means of suitable gears or belts, and continued until the operation is completed. The time occupied in each operation will vary with the various kinds of ore, but from six to eight hours will be found sufficient. The experience gained in working a few panfuls will determine the time necessary to complete the crystallization.

After crystallization has been completed in the pan, the whole mass is drawn off, and the pan is ready for another operation.

The pulp is now put into the amalgamator, shown in Sheet No. 2, which is made as follows: I take a wooden or iron cylinder, or barrel, A, of suitable size, running on a hollow shaft, B. The pulp is introduced into the barrel through a suitable opening, C, with the proper quantity of mercury; close the barrel perfectly tight, then give it very slow motion, by belt or otherwise, for from four to six hours.

After the amalgamation is completed, the amalgam is separated from the pulp by the introduction of a stream of water through the hollow shaft B, by means of the stop-cock D. The pulp being run into cisterns running lengthwise east and west, a plate of suitable metal is put in each end, and these plates connected by a wire outside the cistern. Here it is to remain as long as convenient, or as long as any remaining metals crystallize. This mass may then again be subjected to the action of mercury in the amalgamator.

What I claim as my invention and device, and desire to secure by Letters Patent, is—

1. The mode herein described of collecting gold, silver, and copper from their ores, by the action of independent currents of electricity, in crystallizing the metals in an insulated pan;
2. The amalgamating process, with mercury or any other suitable substance, in an insulated pan or barrel, or other amalgamator.
3. The mode herein described of forming and applying the battery in the pan, or any other, substantially equivalent.
4. The mode of the amalgamation of gold and silver with mercury in an insulated vessel, pan, barrel, or any other, substantially equivalent.
5. The stationary battery in the cisterns, in the form described, or any other, substantially equivalent.
6. Using, for the purposes herein named, the aforesaid machinery and appliances, or any other, substantially the same, in which the same principle is used or involved.

JOHN CORSON.

Witnesses:

T. C. CONNOLLY,  
H. GARRETT.